

# UNITED STATES PATENT OFFICE.

FRANZ VON KÜGELGEN, OF HOLCOMBS ROCK, VIRGINIA, AND GEORGE O. SEWARD, OF NEW YORK, N. Y.

## PROCESS OF ELECTROLYZING AQUEOUS STANNIC-CHLORID SOLUTIONS.

No. 883,141.

Specification of Letters Patent.

Patented March 24, 1908.

Application filed June 10, 1907. Serial No. 378,296.

*To all whom it may concern:*

Be it known that we, FRANZ VON KÜGELGEN, a subject of the Emperor of Germany, residing at Holcombs Rock, Virginia, and GEORGE O. SEWARD, a citizen of the United States, residing at New York city, New York, have invented certain new and useful Improvements in Processes of Electrolyzing Aqueous Stannic - Chlorid Solutions, of which the following is a specification.

In detinning tin-plate scrap by the action of anhydrous chlorin, the tin is recovered as liquid stannic chlorid. This product may be effectively decomposed into tin and chlorin by dissolving it in water and electrolyzing the aqueous solution in a diaphragm cell, with insoluble anodes. Such electrolysis proceeds smoothly at first, but after a time the anolyte becomes basic and the catholyte acid, decreasing the current efficiency, while a gelatinous precipitate may deposit in the anode compartment. This result is due to the fact that stannic chlorid is partially hydrolyzed by water, with the production of stannic hydroxid and hydrochloric acid, which are therefore present in the electrolyte. The difference in the ionic velocities causes the concentration of the base and acid in the cell compartments to gradually change during electrolysis, until the amount of stannic hydroxid in the anode compartment is in excess of that which will remain in solution in the hydrated stannic chlorid.

According to the present process, an aqueous solution of stannic chlorid is electrolyzed by placing it in the cathode compartment of a diaphragm cell, while an aqueous solution containing primarily hydrochloric acid is used in the anode compartment. The catholyte preferably consists of a stannic chlorid solution having a specific gravity of about 1.2; the anolyte of a twenty per cent. hydrochloric acid solution, which may contain a small amount of stannic chlorid. The cell may have walls of slate, a diaphragm of porous earthenware, anodes of graphite and cathodes of sheet tin. The preferred current density at the cathode is 4.2 amperes per square decimeter. As the electrolysis proceeds, the relatively high ionic velocity of the hydrogen cation causes a gradual transfer of hydrochloric acid from the anode to the cathode compartment, until finally the current efficiency begins to notably drop.

At this stage the catholyte may contain about eighteen per cent. of hydrochloric acid and a little stannic chlorid. Both solutions are thereupon removed from the cell and the old catholyte is transferred to the anode compartment, its hydrochloric acid content being brought up to twenty per cent. by the addition of acid. Stannic chlorid is added to the old anolyte until its specific gravity rises to 1.2 and it is then placed in the cathode compartment. The initial cell - conditions are thereby restored and the electrolysis is resumed. The presence of some stannic chlorid in the anolyte is unobjectionable, no stannic hydroxid being formed, therefrom on account of the excess of hydrochloric acid present. During the electrolysis, both solutions may be partially regenerated by the addition of stannic chlorid and hydrochloric acid to the catholyte and anolyte, respectively, thus extending the working period.

We claim:

1. The process of electrolyzing aqueous tin chlorid solutions, which consists in passing an electric current successively through a hydrochloric acid anode solution and a tin chlorid cathode solution, until a considerable percentage of the hydrochloric acid has passed into said cathode solution, then adding tin chlorid to said anode solution and passing an electric current through the two solutions in the opposite direction.

2. The process of electrolyzing aqueous tin chlorid solutions, which consists in passing an electric current successively through an anode solution containing about twenty per cent. of hydrochloric acid and a cathode solution of tin chlorid, until a considerable percentage of the hydrochloric acid has passed into said cathode solution, then adding tin chlorid to said anode solution and passing an electric current through the two solutions in the opposite direction.

In testimony whereof, we affix our signatures in presence of witnesses.

FRANZ VON KÜGELGEN.  
GEORGE O. SEWARD.

Witnesses as to the signature of Franz von Kügelgen:

HARRY RILEY LEE,  
J. H. WEBB.

Witnesses as to the signature of George O. Seward:

JUSTIN C. WALKER,  
GEO. F. SEWARD.